



US009353431B2

(12) **United States Patent**  
**Hatta**

(10) **Patent No.:** **US 9,353,431 B2**  
(45) **Date of Patent:** **May 31, 2016**

(54) **HIGH-STRENGTH ALUMINUM ALLOY MATERIAL AND PROCESS FOR PRODUCING THE SAME**

(75) Inventor: **Hiidenori Hatta**, Aichi (JP)

(73) Assignee: **UACJ CORPORATION**, Tokyo (JP)

(\*) Notice: Subject to any disclaimer, the term of this patent is extended or adjusted under 35 U.S.C. 154(b) by 172 days.

(21) Appl. No.: **14/128,435**

(22) PCT Filed: **Aug. 18, 2011**

(86) PCT No.: **PCT/JP2011/068675**

§ 371 (c)(1),  
(2), (4) Date: **Dec. 20, 2013**

(87) PCT Pub. No.: **WO2012/176345**

PCT Pub. Date: **Dec. 27, 2012**

(65) **Prior Publication Data**

US 2014/0124103 A1 May 8, 2014

(30) **Foreign Application Priority Data**

Jun. 23, 2011 (JP) ..... 2011-139715

(51) **Int. Cl.**

**C22C 21/10** (2006.01)  
**C22F 1/053** (2006.01)

(Continued)

(52) **U.S. Cl.**

CPC ..... **C22F 1/053** (2013.01); **B21C 23/002** (2013.01); **C22C 21/00** (2013.01); **C22C 21/10** (2013.01); **C22F 1/00** (2013.01); **C22F 1/04** (2013.01)

(58) **Field of Classification Search**

CPC ..... C22C 21/10; C22F 1/053

USPC ..... 148/415, 417, 439, 440, 690, 694;  
420/532, 541  
See application file for complete search history.

(56)

**References Cited**

**U.S. PATENT DOCUMENTS**

7,018,489 B2 3/2006 Bennion et al.  
8,105,449 B2 1/2012 Yoshida et al.

(Continued)

**FOREIGN PATENT DOCUMENTS**

CN 1692174 A 11/2005  
CN 1940106 A 4/2007

(Continued)

**OTHER PUBLICATIONS**

English translation of International Preliminary Report on Patentability for parent application No. PCT/JP2012/068675.

(Continued)

*Primary Examiner* — Brian Walck

(74) *Attorney, Agent, or Firm* — J-Tek Law PLLC; Jeffrey D. Tekanic; Scott T. Wakeman

(57) **ABSTRACT**

A high-strength aluminum material having a chemical composition which includes Zn: more than 7.2% (mass %, the same applies hereafter) and 8.7% or less, Mg: 1.3% or more and 2.1% or less, Cu: less than 0.50%, Fe: 0.30% or less, Si: 0.30% or less, Mn: less than 0.05%, Cr: 0.20% or less; Zr: less than 0.05%, Ti: 0.001% or more and 0.05% or less, the balance being Al and unavoidable impurities, is provided. It has a proof stress of 350 MPa or more, and a metallographic structure formed of a recrystallized structure. The recrystallized structure is comprised of crystal grains having an average particle diameter of 500  $\mu\text{m}$  or less, and a crystal grain length in a direction parallel to a hot working direction is 0.5 to 4 times as long as a crystal grain length in a direction perpendicular to the hot working direction.

**20 Claims, 1 Drawing Sheet**



|                      |           |  |    |               |        |  |
|----------------------|-----------|--|----|---------------|--------|--|
| (51) <b>Int. Cl.</b> |           |  |    |               |        |  |
| <i>C22C 21/00</i>    | (2006.01) |  | JP | 2007119904 A  | 5/2007 |  |
| <i>C22F 1/00</i>     | (2006.01) |  | JP | 2010159489 A  | 7/2010 |  |
| <i>C22F 1/04</i>     | (2006.01) |  | WO | 2004046402 A2 | 6/2004 |  |
| <i>B21C 23/00</i>    | (2006.01) |  | WO | 2007009616 A1 | 1/2007 |  |
|                      |           |  | WO | 2008003506 A2 | 1/2008 |  |
|                      |           |  | WO | 2009024601 A1 | 2/2009 |  |

(56) **References Cited**

## U.S. PATENT DOCUMENTS

|                  |         |                 |            |
|------------------|---------|-----------------|------------|
| 2004/0056075 A1  | 3/2004  | Gheorghe        |            |
| 2004/0099352 A1  | 5/2004  | Gheorghe et al. |            |
| 2005/0236075 A1  | 10/2005 | Gheorghe et al. |            |
| 2006/0016523 A1  | 1/2006  | Dif et al.      |            |
| 2006/0157172 A1  | 7/2006  | Fischer et al.  |            |
| 2007/0029016 A1  | 2/2007  | Gheorghe        |            |
| 2007/0074791 A1  | 4/2007  | Yoshida et al.  |            |
| 2007/0151636 A1* | 7/2007  | Buerger .....   | C22C 21/10 |
|                  |         |                 | 148/552    |
| 2007/0187007 A1  | 8/2007  | Gheorghe et al. |            |
| 2008/0299000 A1  | 12/2008 | Gheorghe et al. |            |
| 2014/0096878 A1  | 4/2014  | Hatta et al.    |            |
| 2014/0246127 A1  | 9/2014  | Hatta           |            |

## FOREIGN PATENT DOCUMENTS

|    |              |         |  |
|----|--------------|---------|--|
| EP | 0462055 A1   | 12/1991 |  |
| JP | S60194041 A  | 10/1985 |  |
| JP | H06128678 A  | 5/1994  |  |
| JP | H06330264 A  | 11/1994 |  |
| JP | 2000119782 A | 4/2000  |  |
| JP | 2001355032 A | 12/2001 |  |

## OTHER PUBLICATIONS

English translation of International Search Report for parent application No. PCT/JP2012/068675.

Office Action from the Chinese Patent Office dated Feb. 27, 2015 in related Chinese application No. 2011800718596, and translation of substantive portions thereof.

Office Action from the Korean Patent Office mailed Sep. 5, 2015 in related Korean patent application No. 10-2014-7001906, including translation thereof.

Office Action from the Korean Patent Office mailed Sep. 5, 2015 in related Korean patent application No. 10-2014-7001916, including translation thereof.

English translation of International Preliminary Report on Patentability from counterpart PCT application No. PCT/JP2011/068675. English translation of International Search Report from counterpart PCT application No. PCT/JP2011/068675.

Second Office Action from the Chinese Patent Office dated Jan. 7, 2016 in related Chinese application No. 201280036669.5, and machine translation thereof.

Second Preliminary Amendment filed on Mar. 3, 2016 in U.S. Appl. No. 14/349,239.

\* cited by examiner

FIG. 1



FIG. 2



## 1

**HIGH-STRENGTH ALUMINUM ALLOY  
MATERIAL AND PROCESS FOR  
PRODUCING THE SAME**

## CROSS-REFERENCE

This application is the US national stage of International Patent Application No. PCT/JP2011/068675 filed on Aug. 18, 2011, which claims priority to Japanese Patent Application No. 2011-139715, filed on Jun. 23, 2011.

## TECHNICAL FIELD

The present invention relates to a high-strength aluminum alloy material that can be used at portions of, e.g., transport machines, sporting goods, machine components, etc., where both strength characteristics and appearance characteristics are considered to be important.

## BACKGROUND ART

High-strength and lightweight aluminum alloys are being increasingly employed as materials for use in applications wherein both strength characteristics and appearance characteristics are considered to be important, such as transport machines, sporting goods and machine components. For these applications, because durability is required, there is a desire for aluminum alloys having a proof stress of 350 MPa or more.

7000-series aluminum alloys obtained by adding Zn and Mg to aluminum are known as aluminum alloys which exhibit such high strength. 7000-series aluminum alloys exhibit high strength due to age-precipitation of Al—Mg—Zn-based precipitates. Also, among 7000-series aluminum alloys, those to which Cu has been added in addition to Zn and Mg exhibit the highest strength among the aluminum alloys.

7000-Series aluminum alloys are produced, for example, by hot extrusion, and are used in transport equipment such as aircraft and vehicles, sporting goods and machine components which are required to have high strength. In case they will be used in such applications, the required characteristics include, in addition to strength, resistance to stress corrosion cracking, impact absorption and ductility. For example, the aluminum alloy extruded material described in Patent Document 1 has been proposed as an example of an aluminum alloy that satisfies the above-mentioned characteristics.

## PRIOR ART DOCUMENT

## Patent Document

Patent Document 1: JP 2007-119904 A

## SUMMARY OF THE INVENTION

However, in 7000-series aluminum alloys having a high proof stress produced within a conventional elemental range by a conventional manufacturing process, for example, when anodization, etc. is performed to prevent surface scratching, there is a problem of the appearance in that streak patterns may appear on the surface.

Also, after performing the surface treatment such as anodization, the above-described aluminum alloys are desired to have a silver color in order to engender a luxurious impression. However, when anodizing is performed on the above-described conventional 7000-series aluminum alloys, there

## 2

has been a problem of appearance in that the surface would be strongly tinged with a yellowish color tone.

Thus, the above-described conventional 7000-series aluminum alloys have been difficult to use since the streak patterns and the changes in color tone appearing after the surface treatment have caused surface quality problems.

The present invention has been made in light of such circumstances, and an object of the invention is to provide a high-strength aluminum alloy material having an excellent surface quality and a process for producing the same.

One aspect of the present invention is a high-strength aluminum alloy material having:

15 a chemical composition which includes Zn: more than 7.2% (mass %, the same applies hereafter) and 8.7% or less, Mg: 1.3% or more and 2.1% or less, Cu: less than 0.50%, Fe: 0.30% or less, Si: 0.30% or less, Mn: less than 0.05%, Cr: 0.20% or less, Zr: less than 0.05%, Ti: 0.001% or more and 0.05% or less, the balance being Al and unavoidable impurities;

20 it has a proof stress of 350 MPa or more, and a metallographic structure comprised of a recrystallized structure.

Another aspect of the present invention is a manufacturing 25 method of a high-strength aluminum alloy material, which includes:

30 preparing an ingot having a chemical composition which includes Zn: more than 7.2% (mass %, the same applies hereafter) and 8.7% or less, Mg: 1.3% or more and 2.1% or less, Cu: less than 0.50%, Fe: 0.30% or less, Si: 0.30% or less, Mn: less than 0.05%, Cr: 0.20% or less; Zr: less than 0.05%, Ti: 0.001% or more and 0.05% or less, the balance being Al and unavoidable impurities;

35 performing a homogenization treatment that heats the ingot at a temperature of higher than 540° C. and 580° C. or lower for 1 hour to 24 hours;

40 subsequently, forming a wrought material by performing hot working on the ingot in a state where the temperature of the ingot at the beginning of the working is 440° C. to 560° C.;

while at 400° C. or higher, performing a quenching treatment that cools the wrought material to 150° C. or lower;

cooling the temperature of the wrought material to room 45 temperature by said quenching treatment or by a subsequent cooling; and

thereafter, performing an artificial aging treatment that heats it at a temperature of 100° C. to 170° C. for 5 hours to 30 hours.

The above-described high-strength aluminum alloy material has the above-described specific chemical composition.

50 Therefore, the material has a proof stress equivalent to that of the conventional 7000-series aluminum alloy materials, can also suppress, for example, changes in color tone that occur after a surface treatment and can provide a good surface quality.

55 Also, the high-strength aluminum alloy material has a proof stress of 350 MPa or more. Therefore, the material can relatively easily satisfy the requirements for strength as a material for use in applications wherein both of strength characteristics and appearance are considered to be important.

60 Further, the metallographic structure of the high-strength aluminum alloy material is comprised of a recrystallized structure. Therefore, it is possible to suppress, for example, the generation of streak patterns due to fibrous structures after the surface treatment and to obtain a good surface quality.

65 As described above, the high-strength aluminum material is superior in both strength and surface quality.

Next, in the above-described process for producing a high-strength aluminum alloy material, the high-strength aluminum alloy material is produced using the above-described specific treatment temperature, treatment time and treatment procedures. In this way, the high-strength aluminum alloy material can be easily obtained.

#### BRIEF DESCRIPTION OF THE DRAWINGS

FIG. 1 shows a photograph of the recrystallized structure of Sample No. 1 in Example 1.

FIG. 2 shows a photograph of the fibrous structure of Sample No. 18 in Example 1.

#### MODES FOR CARRYING OUT THE INVENTION

The high-strength aluminum alloy material contains both more than 7.2% and 8.7% or less of Zn and 1.3% or more and 2.1% or less of Mg. Due to coexisting in the aluminum alloy, Zn and Mg precipitate the  $\eta'$  phase. Therefore, the above-mentioned high-strength aluminum alloy material that contains both has increased strength due to enhanced precipitation.

If the Zn content is 7.2% or less, the strength improving effect will be low since the precipitated amount of the  $\eta'$  phase is small. Therefore, the Zn content is preferably more than 7.2%, more preferably 7.5% or more. On the other hand, if the Zn content exceeds 8.7%, productivity is reduced since the hot workability deteriorates. Therefore, the Zn content is preferably 8.7% or less, more preferably 8.5% or less.

If the Mg content is less than 1.3%, the strength improving effect will be low since the precipitated amount of the  $\eta'$  phase is small. On the other hand, if the Mg content exceeds 2.1%, productivity is reduced since the hot workability deteriorates.

Furthermore, in the above-described chemical composition, the content of Cu is restricted to 0.50% or less. Cu may be mixed in the aluminum alloy material when a recycled material is used as a raw material. If Cu is contained in the aluminum alloy material, the strength of the material increases by this effect, although for example the luster after chemical polishing is reduced and the color tone is changed into yellow by anodization, whereby the surface quality deteriorates. Such a deterioration of the surface quality by reduction of the luster or changing of the color tone can be avoided by restricting the content of Cu to 0.50% or less, preferably to 0.20% or less.

Furthermore, in the above-described chemical composition, the respective contents are each restricted as follows: Fe to 0.30% or less, Si to 0.30% or less, Mn to less than 0.05%, Cr to 0.20% or less and Zr to less than 0.05%. Fe and Si are components which are likely to be mixed as impurities in an aluminum base metal, and Mn, Cr and Zr are components which are likely to be mixed when a recycled material is used.

From among the above-mentioned five components, Fe, Si and Mn have the effect of suppressing recrystallization by respectively forming AlMn-based, AlMnFe-based and AlMnFeSi-based intermetallic compounds in combination with Al. Also, Cr and Zr have the effect of suppressing recrystallization by respectively forming AlCr-based and AlZr-based intermetallic compounds. Therefore, the generation of the recrystallized structure is suppressed when the above-mentioned five components are excessively mixed in the high-strength aluminum alloy material and instead, a fibrous structure is easily generated. When (a) fibrous structure(s) is (are) present, streak patterns due to the fibrous structure(s) are likely to occur on the surface after anodization and the surface quality is likely to deteriorate.

The deterioration in surface quality caused by such streak patterns can be suppressed by respectively restricting as follows: Fe to 0.30% or less, Si to 0.30% or less, Mn to less than 0.05%, Cr to 0.20% or less and Zr to less than 0.05%.

Furthermore, the high-strength aluminum alloy material contains 0.001% or more and 0.05% or less of Ti. When added to an aluminum alloy material, Ti has an effect of making the ingot structure fine. Since the ingot structure becomes finer, a higher luster without spots can be obtained, and the surface quality can be improved by incorporating Ti.

If the Ti content is less than 0.001%, the ingot structure is not made sufficiently fine. Therefore, spots may appear on the luster of the high-strength aluminum alloy material. Furthermore, if the Ti content is more than 0.05%, dot-like defects are easily generated, for example, due to an AlTi-based intermetallic compound formed in combination with Al, so that the surface quality is likely to deteriorate.

Further, the high-strength aluminum alloy material has a proof stress, as defined in JIS 22241 (1506892-1), of 350 MPa or more. Due to this, it is possible to relatively easily obtain strength characteristics which enable thinning for weight reduction.

Further, the high-strength aluminum alloy material has a metallographic structure comprised of the granular recrystallized structure. Since an aluminum alloy material produced by performing hot working normally has a metallographic structure composed of (a) fibrous structure(s), (a) streak pattern(s) is (are) likely to appear on the luster of the surface or the like, resulting in a deteriorated surface quality. On the other hand, in the above-mentioned high-strength aluminum alloy material, the metallographic structure is comprised of the recrystallized structure, and thus no streak patterns appear on the surface, thereby providing a good surface quality.

In addition, the metallographic structure can be confirmed, for example, by performing electrolytic polishing on the surface of the aluminum material and by observing the resulting surface using polarized light microscopy.

Furthermore, the recrystallized structure includes crystal grains that have an average particle diameter of 500  $\mu\text{m}$  or less, and a crystal grain length in a direction parallel to the hot working direction is 0.5 to 4 times as long as the crystal grain length in a direction perpendicular to the hot working direction. If the average particle diameter of the crystal grains exceeds 500  $\mu\text{m}$ , the crystal grains become excessively coarse. Therefore, after a surface treatment such as anodization, spots are easily generated on the surface, so that the surface quality is likely to deteriorate. Therefore, a smaller average particle diameter of the crystal grains is better. However, if the average particle diameter is less than 50  $\mu\text{m}$ , (a) fibrous structure(s) is (are) likely to remain between the above-mentioned crystal grains. Thus, the average particle diameter of the crystal grains is preferably 500  $\mu\text{m}$  or less, more preferably 50  $\mu\text{m}$  or more and 500  $\mu\text{m}$  or less in order to obtain a good surface quality.

Furthermore, if the aspect ratio of the above crystal grains (which refers to the ratio of the crystal grain length in a direction parallel to the hot working direction to the crystal grain length in a direction perpendicular to the hot working direction) exceeds 4, (a) streak pattern(s) is (are) likely to appear on the surface after a surface treatment such as anodization. On the other hand, it is difficult to obtain crystal grains having an aspect ratio of less than 0.5 by using most manufacturing equipment.

Furthermore, the recrystallized structure is preferably a recrystallized structure generated during hot working.

Recrystallized structures can be classified into dynamic recrystallized structures and static recrystallized structures

depending on their production process; the recrystallized structures generated during the above-described hot working are referred to as dynamic recrystallized structures. On the other hand, static recrystallized structures refer to those generated by adding heat treatment steps, such as solution heat treatment or annealing treatment, after the hot working or cold working. While the above-described problem can be solved by either recrystallized structure, in the case of the dynamic recrystallized structure, it can be easily produced since the production becomes simpler.

Next, the process for producing a high-strength aluminum alloy material involves a homogenization treatment wherein an ingot having the above-described chemical composition is heated at a temperature of higher than 540° C. and 580° C. or lower for a period of 1 hour or more and 24 hours or less.

If the heating temperature of the homogenization treatment is 540° C. or lower, the homogenization of the ingot segregation layer will be insufficient, resulting in a coarsening of crystal grains, the formation of (a) non-uniform crystalline structure(s) and the like, so that the surface quality of the finally-obtained alloy material deteriorates. On the other hand, if the heating temperature is higher than 580° C., the ingot is likely to locally melt, whereby the manufacturing becomes difficult. Thus, the temperature of the homogenization treatment is preferably higher than 540° C. and 580° C. or lower.

Furthermore, if the heating time for the homogenization treatment is less than 1 hour, the homogenization of the ingot segregation layer will be insufficient, so that the final surface quality deteriorates, as with the above case. On the other hand, if the heating time exceeds 24 hours, the ingot segregation layer has already reached a sufficiently homogenized state, so that no further effect can be expected. Therefore, the time for the homogenization treatment is preferably 1 hour or more and 24 hours or less.

The ingot subjected to the homogenization treatment is made into a wrought material by subjecting to hot working. The temperature of the ingot at the beginning of the hot working is set to 440° C. or higher and 560° C. or lower.

If the heating temperature for the ingot before hot working is lower than 440° C., the resistance to deformation is so high that working in a manufacturing facility actually used will be difficult. On the other hand, if the ingot is subjected to hot working after heating up to a temperature higher than 560° C., the ingot locally melts due to heat generation during the hot working and, as a result, hot cracking is likely to occur. Therefore, the temperature of the ingot before hot working is preferably 440° C. or higher and 560° C. or lower.

Further, extrusion working, rolling working and the like can be employed as the hot working.

After the hot treatment, a quenching treatment is performed that cools the wrought material from a temperature of 400° C. or higher to a temperature of 150° C. or lower.

If the temperature of the wrought material before the quenching treatment is lower than 400° C., the quench hardening will be insufficient, and consequently the proof stress of the resulting wrought material may be less than 350 MPa. Furthermore, if the temperature of the wrought material after the quenching treatment exceeds 150° C., the quench hardening will be insufficient, and consequently the proof stress of the resulting wrought material may be less than 350 MPa.

Further, with respect to the quenching treatment, it means a treatment that involves cooling the wrought material by use of a forcible means. For example, fan air cooling, mist cooling, shower cooling or water cooling can be employed as the quenching treatment.

Furthermore, the cooling rate of the quenching treatment may be in the range of 5° C./sec. to 1000° C./sec.

If the cooling rate exceeds 1000° C./sec., the equipment becomes excessive, but nevertheless no commensurate effect can be obtained. On the other hand, if the cooling rate is less than 5° C./sec., the quench hardening will be insufficient, and consequently the proof stress of the resulting wrought material may not reach 350 MPa. Therefore, a faster cooling rate is better, and the cooling rate is preferably 5° C./sec. or more and 1000° C./sec. or less, more preferably 100° C./sec. or more and 1000° C./sec. or less.

Furthermore, the temperature of the wrought material is brought to room temperature after the quenching treatment. The temperature of the wrought material may be brought to room temperature either by the quenching treatment itself or by an additional cooling treatment after the quenching treatment. Since the effect of room temperature aging is developed by bringing the temperature of the wrought material to room temperature, the strength of the wrought material increases.

Further, for example, fan air cooling, mist cooling, shower cooling or water cooling can be employed as the additional cooling treatment, similar to the quenching treatment.

Here, if the wrought material is stored while maintaining its temperature at room temperature, the strength of the wrought material further increases due to the room temperature aging effect. While a longer room temperature aging time increases the strength more in the initial phase, the room temperature aging effect becomes saturated in case the room temperature aging time is 24 hours or more.

Next, the wrought material, which has been cooled to room temperature as described above, is subjected to the artificial aging treatment that includes heating the wrought material at a temperature of 100° C. or more to 170° C. or less for 5 hour to 30 hours. If the artificial aging treatment is carried out under conditions falling outside the above-mentioned temperature range or time range, the proof stress of the resulting wrought material is likely to be less than 350 MPa. Thus, a wrought material having sufficient strength characteristics cannot be easily obtained.

## EMBODIMENTS

### Example 1

An Example relating to the above-described high-strength aluminum alloy material will be described with reference to Tables 1 and 2.

In this Example, samples (Nos. 1 to 24) that varied the chemical composition of the aluminum alloy material, as indicated in Table 1, were prepared according to the same manufacturing conditions, and strength measurements and metallographic structure observations of each sample were performed. Further, after each sample was subjected to a surface treatment, a surface quality evaluation was performed.

Hereinafter, the manufacturing conditions, the strength measuring method and the metallographic structure observing method, as well as the surface treatment method and the surface quality evaluating method of each sample, will be described.

#### <Manufacturing Conditions of the Samples>

Ingots with a diameter of 90 mm comprised of the chemical compositions indicated in Table 1 are cast by semi-continuous casting. Thereafter, the ingots are subjected to a homogenization treatment that heats them at a temperature of 550° C. for 12 hours. Then, the ingots are subjected to hot extrusion in a state where the temperature of the ingots is 520° C.,

thereby forming wrought materials having a width of 150 mm and a thickness of 10 mm. Then, while the temperature of the wrought materials is 505°C., the wrought materials are subjected to a quenching treatment that cools the wrought materials to 100°C. at an average cooling rate of 600°C./sec. The wrought materials subjected to the quenching treatment are cooled to room temperature, and subjected to room temperature aging at room temperature for 24 hours, and thereafter subjected to an artificial aging treatment that heats the wrought materials at a temperature of 150°C. for 12 hours.

<Strength Measuring Method>

Test pieces are collected from the samples by a method in accordance with JIS 22241 (1506892-1) and measurements of the tensile strength, proof stress and elongation are performed. As a result, those exhibiting a proof stress of 350 MPa or more are judged to be acceptable.

<Metallographic Structure Observing Method>

After performing electrolytic polishing on the samples, microscopic images of the sample surfaces are obtained by using a polarizing light microscope having a magnification of 50 to 100. Image analysis is performed on the microscopic images to obtain the average particle diameter of the crystal grains constituting the metallographic structure of the samples, and the aspect ratio. As a result, the samples having an average particle diameter of 500 µm or less and the samples having an aspect ratio ranging from 0.5 to 4.0 are judged to be preferred results.

<Surface Treatment Method>

After buffing the surfaces of the samples that were subjected to the artificial aging treatment, the samples are etched with a sodium hydroxide solution, and then subjected to a de-smutting treatment. The samples subjected to the de-smutting treatment are chemically polished using a phosphoric acid-nitric acid method at a temperature of 90°C. for 1 minute. Then, the samples subjected to chemically-polishing are subjected to anodization at a current density of 150 A/m<sup>2</sup> in a 15% sulfuric acid bath to form 10-µm anodic oxide coatings. Finally, the samples subjected to the anodization are immersed in boiling water to perform a hole-sealing treatment on the anodic oxide coatings.

<Surface Quality Evaluating Method>

The surfaces of the samples subjected to the surface treatment are visually observed. In the visual observation, the samples which did not develop any streak patterns, spotting patterns, dot-like defects or the like on their surfaces are judged to be acceptable.

Then, the color tone of the sample surfaces is measured by a color-difference meter to obtain the respective coordinate values in the L\*a\*b\* color system described in JIS 28729 (1507724-1). As a result, the samples having an L\* value (lightness): 85 to 95, an a\* value (chromaticity of green to red): -2.0 to 0 and a b\* value (chromaticity of blue to yellow): -0.5 to 2.5 are judged to be acceptable.

The evaluation results for each of the samples prepared in the manner as described above are indicated in Table 2. Further, for the samples which were not judged as being acceptable or favorable in the evaluation results, the evaluation results are underlined in Table 2.

As can be seen from Table 2, Samples Nos. 1 to 12 were judged as being acceptable in terms of all the evaluation criteria, and exhibited excellent properties in both strength and surface quality.

As a typical example of a sample having excellent surface quality, FIG. 1 shows the observation result of the metallographic structure of Sample No. 1. The samples having excellent surface quality have a metallographic structure comprised of a granular recrystallized structure, and, at the same

time, do not exhibit any streak patterns even by visual confirmation, are free of spots, and have high luster.

Sample No. 13, the Zn content of which was too low, was judged as being unacceptable in terms of proof stress because the strength improving effect could not sufficiently obtained.

Sample No. 14, the Zn content of which was too high, was poor in hot workability and could not be subjected to hot extrusion with manufacturing facilities actually used.

Sample No. 15, the Mg content of which was too low, was 10 judged as being unacceptable in terms of proof stress because the strength improving effect could not sufficiently obtained.

Sample No. 16, the Mg content of which was too high, was poor in hot workability and could not be subjected to hot extrusion with actually used facilities.

15 Sample No. 17, the Cu content of which was too high, was judged as being unacceptable because its surface became yellowish in color.

Sample No. 18, the Fe content of which was too high, was 20 judged as being unacceptable because fibrous structures were formed and, as a result, streak patterns were visually recognized on its surface.

FIG. 2 shows the observation result of the metallographic structure of Sample No. 18 as a typical example of the samples in which streak patterns were visually recognized, 25 among the samples judged as being unacceptable in terms of surface quality. The samples in which streak patterns were visually recognized have a metallographic structure comprised of fibrous structures as can be seen from FIG. 2.

Sample No. 19, the Si content of which was too high, was 30 judged as being unacceptable because fibrous structures were formed, and as a result, streak patterns were visually recognized on its surface. In addition, its surface became yellowish in color.

Sample No. 20, the Mn content of which was too high, was 35 judged as being unacceptable because fibrous structures were formed, and as a result, streak patterns were visually recognized on its surface.

Sample No. 21, the Cr content of which was too high, was 40 judged as being unacceptable because fibrous structures were formed, and as a result, streak patterns were visually recognized on its surface. In addition, its surface became yellowish in color.

Sample No. 22, the Zr content of which was too high, was 45 judged as being unacceptable because fibrous structures were formed, and as a result, streak patterns were visually recognized on its surface.

Sample No. 23, the Ti content of which was too low, was 50 judged as being unacceptable because a spotting pattern appeared due to a coarse ingot structure.

Sample No. 24, the Ti content of which was too high, was 55 judged as being unacceptable because intermetallic compounds was formed in combination with Al, and as a result, dot-like defects were visually recognized on its surface.

Example 2

Next, an Example relating to the above-described process for producing a high-strength aluminum alloy material will be described with reference to Tables 3 and 5.

60 In this Example, samples (Nos. A to X) were prepared from the aluminum alloy material having the chemical composition indicated in Table 3 according to the manufacturing conditions that varied as indicated in Table 4, and strength measurements and metallographic structure observations of each sample were performed. Further, after each sample was subjected to a surface treatment, a surface quality evaluation was performed.

Hereinafter, the conditions for manufacturing the respective samples will be described in detail. Further, the strength measuring method, the metallographic structure observing method, the surface treatment method and the surface quality evaluating method for the respective samples were the same as described above in Example 1.

<Manufacturing Conditions of the Samples>

Ingots with a diameter of 90 mm comprised of the chemical composition indicated in Table 3 are cast using a semi-continuous casting technique. Thereafter, the ingots are subjected to a homogenization treatment, a hot extrusion, a quenching treatment, and an artificial aging treatment in this order using the combinations of treatment temperature, treatment time and cooling rate as indicated in Table 4 to obtain samples. Further, the "room temperature aging time" indicated in Table 4 corresponds to the period of time from when the wrought material reached room temperature after the quenching treatment until the artificial aging treatment was carried out.

The evaluation results for each of the samples prepared as described above are indicated in Table 5. Further, for the samples which were not judged as being acceptable or preferable in the respective evaluation results, the evaluation results therefor are underlined in Table 5.

As can be seen from Table 5, Samples Nos. A to 0 were judged as being acceptable in terms of all the evaluation criteria, and exhibited excellent properties in both strength and surface quality.

Sample P, prepared by subjecting to the homogenization treatment at a too low heating temperature, was judged as being unacceptable because the proof stress is less than 350 MPa. At the same time, the crystal grains became coarse, and also a spotty pattern was visually recognized on its surface.

Sample Q, prepared by subjecting to the homogenization treatment for a too short time, was judged as being unacceptable because the proof stress is less than 350 MPa. At the same time, the crystal grains became coarse, and also a spotty pattern was visually recognized on its surface.

Sample R, prepared by heating an ingot at a too high temperature before hot extrusion working, partially melted during extrusion working, and as a result, caused hot working cracks, and thus could not be subjected to the quenching treatment and the subsequent treatments.

Sample S, prepared by subjecting to the quenching treatment at a too low cooling rate, was judged as being unacceptable because the proof stress is less than 350 MPa due to insufficient quenching.

Sample T, prepared from a wrought material having a too high temperature after the quenching treatment, was judged as being unacceptable because the proof stress is less than 350 MPa due to insufficient quenching.

Sample U, prepared by subjecting to the artificial aging treatment at a too low heating temperature, was judged as being unacceptable because the proof stress is less than 350 MPa due to insufficient quenching.

Sample V, prepared by subjecting to the artificial aging treatment at a too high heating temperature, was judged as being unacceptable because the proof stress is less than 350 MPa due to over-aging.

Sample W, prepared by subjecting to the artificial aging treatment for a too short time, was judged as being unacceptable because the proof stress is less than 350 MPa due to insufficient quenching.

Sample X, prepared by subjecting to the artificial aging treatment for a too long time, was judged as being unacceptable because the proof stress is less than 350 MPa due to over-aging.

TABLE 1

| Sample No. | Zn (%)      | Mg (%)      | Cu (%)      | Fe (%)      | Si (%)      | Mn (%)      | Cr (%)      | Zr (%)      | Ti (%)        | Al (%) |
|------------|-------------|-------------|-------------|-------------|-------------|-------------|-------------|-------------|---------------|--------|
| 1          | <u>7.25</u> | 1.72        | 0.06        | 0.21        | 0.1         | 0.01        | 0.05        | 0.01        | 0.01          | bal    |
| 2          | <u>8.67</u> | 1.68        | 0.06        | 0.17        | 0.08        | 0.01        | 0.07        | 0.01        | 0.02          | bal    |
| 3          | 7.51        | <u>1.32</u> | 0.05        | 0.18        | 0.13        | 0.02        | 0.03        | 0.01        | 0.01          | bal    |
| 4          | 8.01        | <u>2.08</u> | 0.11        | 0.18        | 0.17        | 0.01        | 0.07        | 0.02        | 0.007         | bal    |
| 5          | 7.58        | 1.75        | <u>0.48</u> | 0.17        | 0.17        | 0.01        | 0.05        | 0.01        | 0.008         | bal    |
| 6          | 7.59        | 1.73        | 0.17        | <u>0.29</u> | 0.18        | 0.01        | 0.11        | 0.01        | 0.02          | bal    |
| 7          | 7.61        | 1.77        | 0.12        | 0.2         | <u>0.28</u> | 0.02        | 0.13        | 0.01        | 0.01          | bal    |
| 8          | 7.92        | 1.79        | 0.07        | 0.19        | 0.09        | <u>0.04</u> | 0.1         | 0.02        | 0.009         | bal    |
| 9          | 7.93        | 1.78        | 0.05        | 0.18        | 0.17        | 0.03        | <u>0.17</u> | 0.03        | 0.01          | bal    |
| 10         | 7.92        | 1.79        | 0.03        | 0.19        | 0.2         | 0.01        | 0.07        | <u>0.04</u> | 0.01          | bal    |
| 11         | 7.94        | 1.76        | 0.05        | 0.17        | 0.17        | 0.01        | 0.08        | 0.01        | <u>0.002</u>  | bal    |
| 12         | 7.93        | 1.77        | 0.04        | 0.18        | 0.18        | 0.02        | 0.02        | 0.01        | <u>0.04</u>   | bal    |
| 13         | <u>7.2</u>  | 1.65        | 0.05        | 0.18        | 0.09        | 0.01        | 0.08        | 0.01        | 0.008         | bal    |
| 14         | <u>8.77</u> | 1.58        | 0.05        | 0.19        | 0.11        | 0.01        | 0.05        | 0.01        | 0.01          | bal    |
| 15         | 7.67        | <u>1.26</u> | 0.06        | 0.17        | 0.1         | 0.01        | 0.05        | 0.02        | 0.01          | bal    |
| 16         | 7.55        | <u>2.16</u> | 0.11        | 0.12        | 0.15        | 0.01        | 0.06        | 0.01        | 0.01          | bal    |
| 17         | 8.12        | 1.61        | <u>0.58</u> | 0.21        | 0.06        | 0.01        | 0.07        | 0.01        | 0.02          | bal    |
| 18         | 7.52        | 1.71        | 0.06        | <u>0.33</u> | 0.19        | 0.01        | 0.08        | 0.03        | 0.009         | bal    |
| 19         | 7.39        | 1.7         | 0.02        | 0.23        | <u>0.35</u> | 0.02        | 0.05        | 0.01        | 0.02          | bal    |
| 20         | 7.28        | 1.69        | 0.03        | 0.18        | 0.11        | <u>0.05</u> | 0.05        | 0.01        | 0.01          | bal    |
| 21         | 7.88        | 1.74        | 0.03        | 0.19        | 0.15        | 0.02        | <u>0.24</u> | 0.01        | 0.01          | bal    |
| 22         | 7.67        | 1.75        | 0.03        | 0.18        | 0.13        | 0.02        | 0.11        | <u>0.05</u> | 0.01          | bal    |
| 23         | 7.54        | 1.69        | 0.04        | 0.19        | 0.1         | 0.01        | 0.13        | 0.02        | <u>0.0007</u> | bal    |
| 24         | 7.86        | 1.73        | 0.03        | 0.19        | 0.13        | 0.01        | 0.08        | 0.01        | <u>0.06</u>   | bal    |

TABLE 2

| Sample No. | Strength Test          |                    |                | Observation of Metallographic Structure                       |              |                              | Evaluation of Surface Quality |          |          |
|------------|------------------------|--------------------|----------------|---------------------------------------------------------------|--------------|------------------------------|-------------------------------|----------|----------|
|            | Tensile Strength (MPa) | Proof Stress (MPa) | Elongation (%) | Average Particle Diameter of Crystal Grains ( $\mu\text{m}$ ) | Aspect Ratio | Result of Visual Observation | L* value                      | a* value | b* value |
| 1          | 388                    | 354                | 17             | 220                                                           | 1.4          | No pattern                   | 92                            | -0.5     | 0.5      |
| 2          | 545                    | 512                | 13             | 150                                                           | 1            | No pattern                   | 88                            | -1.8     | 0.9      |
| 3          | 391                    | 367                | 18             | 450                                                           | 3.2          | No pattern                   | 91                            | -0.4     | 0.4      |
| 4          | 537                    | 508                | 13             | 150                                                           | 2.8          | No pattern                   | 89                            | -1.8     | 0.9      |
| 5          | 511                    | 483                | 15             | 220                                                           | 1.9          | No pattern                   | 85                            | -2.0     | 2.0      |
| 6          | 487                    | 455                | 16             | 90                                                            | 1.4          | No pattern                   | 94                            | -0.2     | -0.4     |
| 7          | 470                    | 447                | 15             | 110                                                           | 1.6          | No pattern                   | 86                            | -0.5     | 0.7      |
| 8          | 489                    | 452                | 14             | 100                                                           | 1.6          | No pattern                   | 89                            | -1.8     | 1.9      |
| 9          | 480                    | 448                | 16             | 160                                                           | 2.1          | No pattern                   | 86                            | -0.7     | 0.6      |
| 10         | 491                    | 458                | 15             | 55                                                            | 0.7          | No pattern                   | 90                            | -0.9     | 0.7      |
| 11         | 476                    | 444                | 15             | 120                                                           | 1.7          | No pattern                   | 89                            | -0.5     | 0.7      |
| 12         | 486                    | 451                | 15             | 120                                                           | 1.8          | No pattern                   | 89                            | -0.6     | 0.8      |
| 13         | 374                    | 336                | 18             | 520                                                           | 4.3          | No pattern                   | 93                            | -0.6     | 0.3      |
| 14         |                        |                    |                | Out of production due to low extrusion rate                   |              |                              |                               |          |          |
| 15         | 361                    | 329                | 17             | 530                                                           | 4.2          | No pattern                   | 94                            | -0.8     | 0.4      |
| 16         |                        |                    |                | Out of production due to low extrusion rate                   |              |                              |                               |          |          |
| 17         | 515                    | 489                | 15             | 110                                                           | 1.5          | No pattern                   | 81                            | -2.2     | 2.7      |
| 18         | 491                    | 451                | 16             | Not measurable                                                |              | Streak patterns              | 90                            | -1.6     | 0.4      |
|            |                        |                    |                | due to fibrous structure                                      |              | Streak patterns              | 80                            | -1.7     | 2.8      |
| 19         | 480                    | 444                | 16             | Not measurable                                                |              | Streak patterns              | 86                            | -2.1     | 1.5      |
|            |                        |                    |                | due to fibrous structure                                      |              | Streak patterns              | 82                            | -0.3     | 2.6      |
| 20         | 493                    | 458                | 15             | Not measurable                                                |              | Streak patterns              | 87                            | -1.7     | 0.6      |
|            |                        |                    |                | due to fibrous structure                                      |              | Streak patterns              | 88                            | -0.5     | 1.2      |
| 21         | 462                    | 438                | 16             | Not measurable                                                |              | Dot-like defect              | 89                            | -0.4     | 1.1      |
|            |                        |                    |                | due to fibrous structure                                      |              |                              |                               |          |          |
| 22         | 500                    | 461                | 13             | Not measurable                                                |              |                              |                               |          |          |
|            |                        |                    |                | due to fibrous structure                                      |              |                              |                               |          |          |
| 23         | 499                    | 463                | 12             | Not measurable                                                |              |                              |                               |          |          |
|            |                        |                    |                | due to coarse ingot structure                                 |              |                              |                               |          |          |
| 24         | 494                    | 459                | 13             | 110                                                           | 2.8          |                              |                               |          |          |

35

TABLE 3

| Zn (%) | Mg (%) | Cu (%) | Fe (%) | Si (%) | Mn (%) | Cr (%) | Zr (%) | Ti (%) | Al (%) |
|--------|--------|--------|--------|--------|--------|--------|--------|--------|--------|
| 7.86   | 1.73   | 0.05   | 0.21   | 0.17   | 0.01   | 0.03   | 0.01   | 0.008  | bal    |

40

TABLE 4

| Sample No. | Homogenization            |                     | Hot Extrusion                      |     | Quenching Treatment          |              |                                         | Artificial Aging Treatment |                       |                |
|------------|---------------------------|---------------------|------------------------------------|-----|------------------------------|--------------|-----------------------------------------|----------------------------|-----------------------|----------------|
|            | Treatment                 |                     | Ingot                              |     | Temperature before Quenching | Cooling Rate | Temperature immediately after quenching | Temperature Aging Time     | Treatment Temperature | Treatment Time |
|            | Heating Temperature (°C.) | Heating Time (Hour) | Temperature before Extrusion (°C.) |     | (°C./Second)                 | (°C.)        |                                         |                            |                       |                |
| A          | 541                       | 12                  | 502                                | 490 | 230                          | 100          | 24                                      | 136                        | 8                     |                |
| B          | 578                       | 12                  | 497                                | 471 | 150                          | 120          | 24                                      | 129                        | 12                    |                |
| C          | 561                       | 1                   | 500                                | 493 | 220                          | 100          | 48                                      | 134                        | 8                     |                |
| D          | 562                       | 24                  | 501                                | 486 | 460                          | 110          | 48                                      | 133                        | 12                    |                |
| E          | 558                       | 18                  | 442                                | 422 | 350                          | 130          | 120                                     | 134                        | 18                    |                |
| F          | 565                       | 18                  | 556                                | 543 | 260                          | 100          | 120                                     | 130                        | 8                     |                |
| G          | 561                       | 16                  | 498                                | 477 | 5                            | 90           | 120                                     | 138                        | 20                    |                |
| H          | 553                       | 16                  | 488                                | 461 | 970                          | 110          | 144                                     | 131                        | 12                    |                |
| I          | 560                       | 8                   | 503                                | 491 | 60                           | 150          | 144                                     | 133                        | 20                    |                |
| J          | 556                       | 8                   | 502                                | 487 | 90                           | 100          | 0                                       | 129                        | 18                    |                |
| K          | 560                       | 6                   | 501                                | 485 | 550                          | 100          | 240                                     | 136                        | 12                    |                |
| L          | 557                       | 4                   | 495                                | 479 | 160                          | 110          | 120                                     | 104                        | 12                    |                |
| M          | 556                       | 12                  | 502                                | 482 | 310                          | 100          | 120                                     | 167                        | 8                     |                |
| N          | 560                       | 14                  | 503                                | 490 | 180                          | 90           | 72                                      | 130                        | 5                     |                |
| O          | 558                       | 14                  | 498                                | 472 | 330                          | 100          | 72                                      | 131                        | 30                    |                |
| P          | 535                       | 12                  | 498                                | 481 | 150                          | 90           | 24                                      | 130                        | 12                    |                |
| Q          | 555                       | 0.5                 | 503                                | 483 | 190                          | 120          | 24                                      | 130                        | 12                    |                |
| R          | 562                       | 12                  | 564                                |     |                              |              |                                         |                            |                       |                |
| S          | 558                       | 12                  | 505                                | 482 | 4                            | 100          | 24                                      | 131                        | 12                    |                |

Hot working cracking caused by local melting was generated

TABLE 4-continued

| Sample No. | Homogenization            |                     | Hot Extrusion                      | Quenching Treatment |                                    |                           | Artificial Aging Treatment                    |                         |                             |
|------------|---------------------------|---------------------|------------------------------------|---------------------|------------------------------------|---------------------------|-----------------------------------------------|-------------------------|-----------------------------|
|            | Treatment                 |                     |                                    | Ingot               | Temperature before Quenching (°C.) | Cooling Rate (°C./Second) | Temperature immediately after quenching (°C.) | Room Temperature (Hour) | Treatment Temperature (°C.) |
|            | Heating Temperature (°C.) | Heating Time (Hour) | Temperature before Extrusion (°C.) |                     |                                    |                           |                                               |                         |                             |
| T          | 553                       | 12                  | 497                                | 479                 | 50                                 | 170                       | 24                                            | 127                     | 12                          |
| U          | 554                       | 12                  | 500                                | 486                 | 30                                 | 100                       | 24                                            | 90                      | 12                          |
| V          | 558                       | 12                  | 503                                | 491                 | 170                                | 90                        | 24                                            | 175                     | 12                          |
| W          | 562                       | 12                  | 507                                | 492                 | 180                                | 110                       | 24                                            | 131                     | 4                           |
| X          | 561                       | 12                  | 506                                | 492                 | 190                                | 120                       | 24                                            | 135                     | 32                          |

TABLE 5

| Sample No. | Strength Test                                |                    |                | Observation of Metallographic Structure          |              |                              | Evaluation of Surface Quality |          |          |  |
|------------|----------------------------------------------|--------------------|----------------|--------------------------------------------------|--------------|------------------------------|-------------------------------|----------|----------|--|
|            | Tensile Strength (MPa)                       | Proof Stress (MPa) | Elongation (%) | Average Particle Diameter of Crystal Grains (μm) | Aspect Ratio | Result of Visual Observation | L* value                      | a* value | b* value |  |
| A          | 411                                          | 375                | 17             | 460                                              | 3.7          | No pattern                   | 88                            | -1.1     | 0.6      |  |
| B          | 500                                          | 467                | 14             | 110                                              | 1            | No pattern                   | 87                            | -0.9     | 0.8      |  |
| C          | 402                                          | 369                | 18             | 320                                              | 2.8          | No pattern                   | 91                            | -0.8     | 0.7      |  |
| D          | 513                                          | 477                | 13             | 120                                              | 1            | No pattern                   | 89                            | -1.3     | 1.0      |  |
| E          | 391                                          | 364                | 17             | 290                                              | 3.1          | No pattern                   | 93                            | -0.5     | 0.3      |  |
| F          | 507                                          | 473                | 15             | 130                                              | 1.3          | No pattern                   | 86                            | -1.8     | 0.8      |  |
| G          | 393                                          | 357                | 17             | 350                                              | 2.9          | No pattern                   | 92                            | -0.7     | 0.2      |  |
| H          | 511                                          | 488                | 14             | 90                                               | 0.7          | No pattern                   | 87                            | -1.9     | 0.8      |  |
| I          | 396                                          | 361                | 16             | 290                                              | 2.2          | No pattern                   | 93                            | -0.6     | 0.0      |  |
| J          | 403                                          | 373                | 12             | 80                                               | 0.7          | No pattern                   | 85                            | -1.5     | 0.7      |  |
| K          | 521                                          | 490                | 16             | 360                                              | 3.3          | No pattern                   | 94                            | -0.7     | 0.3      |  |
| L          | 392                                          | 358                | 17             | 340                                              | 4            | No pattern                   | 90                            | -0.9     | 0.5      |  |
| M          | 512                                          | 477                | 13             | 80                                               | 0.6          | No pattern                   | 86                            | -1.7     | 1.1      |  |
| N          | 390                                          | 362                | 18             | 280                                              | 2.2          | No pattern                   | 93                            | -0.6     | 0.1      |  |
| O          | 501                                          | 474                | 13             | 70                                               | 0.9          | No pattern                   | 87                            | -1.6     | 1.3      |  |
| P          | 351                                          | 314                | 16             | 620                                              | 5.2          | Spotting pattern             | 92                            | -0.5     | 0.4      |  |
| Q          | 366                                          | 327                | 17             | 550                                              | 4.3          | Spotting pattern             | 91                            | -0.4     | 0.3      |  |
| R          | Hot working cracking caused by local melting |                    |                |                                                  |              |                              |                               |          |          |  |
| S          | 368                                          | 336                | 16             | 260                                              | 2.1          | No pattern                   | 92                            | -0.5     | 0.2      |  |
| T          | 353                                          | 318                | 14             | 210                                              | 1.7          | No pattern                   | 90                            | -0.5     | 0.4      |  |
| U          | 371                                          | 337                | 13             | 130                                              | 1            | No pattern                   | 92                            | -0.7     | 0.6      |  |
| V          | 373                                          | 340                | 16             | 210                                              | 1.5          | No pattern                   | 91                            | -0.5     | 0.2      |  |
| W          | 362                                          | 338                | 14             | 120                                              | 1.2          | No pattern                   | 90                            | -0.6     | 0.5      |  |
| X          | 378                                          | 342                | 15             | 110                                              | 1.4          | No pattern                   | 91                            | -0.6     | 0.6      |  |

The invention claimed is:

1. An aluminum alloy material, comprising in mass percent:

Zn: more than 7.2% and 8.7% or less,

Mg: 1.3% or more and 2.1% or less,

Cu: less than 0.50%,

Fe: 0.30% or less,

Si: 0.30% or less,

Mn: less than 0.05%,

Cr: 0.20% or less,

Zr: less than 0.05%,

Ti: 0.001% or more and 0.05% or less,

the balance being Al and unavoidable impurities;

wherein the aluminum alloy material has a proof stress of 350 MPa or more, and a metallographic structure consisting essentially of a recrystallized structure.

2. The aluminum alloy material according to claim 1, wherein:

the recrystallized structure includes crystal grains having an average particle diameter of 500 μm or less, and

a crystal grain length in a direction parallel to a hot working direction is 0.5 to 4 times as long as a crystal grain length in a direction perpendicular to the hot working direction.

3. The aluminum alloy material according to claim 2, wherein Zn is more than 7.5% and 8.5% or less.

4. The aluminum alloy material according to claim 3, wherein Cu is 0.2% or less.

5. The aluminum alloy material according to claim 4, wherein the crystal grains have an average particle diameter of 50 μm or more.

6. The aluminum alloy material according to claim 5, wherein the recrystallized structure is a granular recrystallized structure.

7. The aluminum alloy material according to claim 1, wherein Zn is more than 7.5% and 8.5% or less.

8. The aluminum alloy material according to claim 1, wherein Cu is 0.2% or less.

9. The aluminum alloy material according to claim 1, wherein the crystal grains have an average particle diameter of 50 μm or more.

**15**

**10.** The aluminum alloy material according to claim 1, wherein the recrystallized structure is a granular recrystallized structure.

**11.** The aluminum alloy material according to claim 1, wherein Zr is 0.04% or less.

**12.** A process for producing the aluminum alloy material according to claim 1, which comprises:

preparing an ingot having a chemical composition which comprises in mass percent Zn: more than 7.2% and 8.7% or less, Mg: 1.3% or more and 2.1% or less, Cu: less than 0.50%, Fe: 0.30% or less, Si: 0.30% or less, Mn: less than 0.05%, Cr: 0.20% or less; Zr: less than 0.05%, Ti: 0.001% or more and 0.05% or less, the balance being Al and unavoidable impurities;

15 performing a homogenization treatment that heats the ingot at a temperature of higher than 540° C. and 580° C. or lower for 1 hour to 24 hours;

subsequently, forming a wrought material by performing hot working on the ingot in a state where the temperature of the ingot at the beginning of the hot working is 440° C. to 560° C.;

20 while the wrought material is still at 400° C. or higher, performing a quenching treatment that cools the wrought material to 150° C. or lower;

cooling the temperature of the wrought material to room 25 temperature by said quenching treatment itself or by an additional cooling treatment; and

thereafter, performing an artificial aging treatment that heats the wrought material at a temperature of 100° C. to 170° C. for 5 hours to 30 hours,

30 wherein the wrought material has a proof stress of 350 MPa or more, and a metallographic structure consisting essentially of a recrystallized structure.

**13.** The process according to claim 12, wherein the quenching treatment is performed at a cooling rate of 5° C./sec. to 35 1000° C./sec.

**14.** The process according to claim 13, wherein the cooling rate is 100° C./sec. or more.

**15.** The process according to claim 14, wherein the hot working involves extrusion or rolling.

**16**

**16.** The process according to claim 15, further comprising anodizing the wrought material after the artificial aging treatment.

**17.** The process according to claim 12, wherein: 5 the homogenization treatment is performed at 550° C. for 12 hours,

the hot working comprises subjecting the ingot to extrusion and is initiated while the temperature of the ingot is at 520° C.,

10 the quenching treatment is initiated while the temperature of the wrought material is at 505° C. and the cooling rate of the quenching treatment is 600° C./sec, and the artificial aging treatment involves heating the wrought material at 150° C. for 12 hours.

**18.** The process according to claim 17, further comprising anodizing the wrought material after the artificial aging treatment.

**19.** The process according to claim 12, further comprising anodizing the wrought material after the artificial aging treatment.

**20.** A process for producing the aluminum alloy material of claim 1, comprising:

homogenizing an ingot having the elemental composition recited in claim 5 at a temperature of higher than 540° C. and 580° C. or lower for at least 1 hour;

hot working the homogenized ingot, the hot working being initiated while the temperature of the homogenized ingot is 440° C. to 560° C.;

quenching hot worked material to 150° C. or lower, the quenching being initiated while the hot worked material is at a temperature of 400° C. or higher,

cooling the hot worked material to room temperature; and subjecting the cooled material to an artificial aging treatment at a temperature of 100° C. to 170° C. for 5 hours to 30 hours,

wherein the aluminum alloy material has a proof stress of 350 MPa or more, and a metallographic structure consisting essentially of a recrystallized structure.

\* \* \* \* \*